

## UNITED STATES PATENT OFFICE

2,146,938

PRODUCTION OF PHOTOGRAPHIC  
EMULSIONS

Bruno Claus, Halle-on-the-Saale, Germany

No Drawing. Application March 18, 1936, Serial  
No. 69,520. In Germany April 5, 1935

8 Claims. (Cl. 95—7)

My invention relates to photographic emulsions and more especially to means whereby emulsions possessing particularly favorable properties can be produced in a particularly simple and effective manner.

As is well known to those skilled in the art, the production of photographic emulsions by first causing the silver halide and more especially silver bromide to be preformed separately and to settle as a sediment and to thereafter emulsifying the silver salt in a binder such as for instance gelatine, offers the advantage, as compared with other modes of preparation of such emulsions, that it avoids the circumstantial, unreliable and time-consuming subsequent washing, whereby the preparation of photographic mixtures of silver halides and gelatine or the like are greatly simplified. Hitherto this mode of proceeding merely allowed producing fine-grained photographic emulsions, which were little sensitive to the action of light and to produce similar emulsions, which are known under the name of peptisation emulsions, with a medium or more coarse grain size appeared impossible.

I have now found that the solution of this problem is of paramount importance since my experiments have shown that peptisation emulsions of the kind aforesaid and more particularly such emulsions of this kind which have been caused to age by adding ammonia, are not only distinguished by the simplicity, with which they can be produced, but also by their high sensitivity to the action of light, which as a rule surpasses the sensitivity of emulsions of the same order of grain size which were produced according to some customary mode of production.

As I have already mentioned above, it was hitherto only possible to produce peptisation emulsions having a fine grain and a sensitivity up to about 14° Din. According to the present invention now I am enabled to produce peptisation emulsions of medium or more coarse grain size and which nevertheless possess a very high sensitivity to light, being in certain cases finer grained than corresponding emulsions of similar sensitivity which were produced according to customary processes.

The new process for the production of peptisation emulsions possessing these desirable properties substantially consists therein, that to a silver halide emulsion, more especially to a silver bromide sediment which may or may not yet have been emulsified in a binder, for instance gelatine, is gradually added during the aging period a silver halide and more especially silver

bromide of a finer grain preformed in the form of a sediment and which may or may not have been emulsified in an emulsion substratum such as for instance gelatine, the mixture thus obtained being subjected to a suitable aging temperature under the action of chemical substances favoring the aging process, such as for instance solutions of ammonia.

In the carrying out of the new process, I may for instance proceed as follows:—

## Example 1

A 10% solution of potassium bromide containing about 0.4% potassium iodide and which may further contain some gelatine is mixed with a solution of nitrate of silver, which solution may also contain some gelatine, the two solutions being mixed in such proportions that in the mixture a slight excess of bromide, for instance amounting to 2%, is present. The silver halide formed in the solution is allowed to settle down as a sediment, which is now washed out. A part of this sediment, say one fifth, is then emulsified in an aqueous gelatine solution containing ammonia (about 3% gelatine and 2% ammonia) and the mixture is now heated up to 50 to 60° C., varying in accordance with the degree of sensitivity of the gelatine used. To the slightly heated mixture is now gradually added some of the washed silver halide sediment and, if necessary, there is also gradually added some ammonia to such an extent that the ammonia which evaporates during the aging period, is replaced to substantially maintain the initial concentration, until the remainder of the silver halide is spent. Now gelatine is added to the mixture of silver halide and gelatine until the emulsion contains sufficient gelatine (about 9%). After the missing gelatine has thus been added, the emulsion may still be kept some time at an elevated temperature without adding ammonia, and then the ammonia still present in the emulsion is cautiously neutralized, for instance by adding citric acid. The emulsion is now ready for pouring.

## Example 2

A 10% potassium bromide solution containing about 0.4% potassium iodide and which may also contain a small proportion of gelatine, is mixed with a solution of nitrate of silver, which may also contain some gelatine. The silver halide formed in the mixture is allowed to settle as a sediment, which is washed out and emulsified in an aqueous 3% solution of gelatine, for instance by adding some ammonia. The emulsion is now divided; to one of the two portions is added some

more ammonia to bring its ammonia contents to about 2%, whereupon this portion is heated to about 55° C. Now some of the remainder of the emulsion is gradually added to the portion treated as above and, if necessary, some more ammonia is added in order to replace the amount of ammonia lost by evaporation. This mode of proceeding is continued until the whole of the emulsion has been added. I now add so much 5 gelatine, that the emulsion contains about 9% gelatine. The mixture may be kept at an elevated temperature for some time without adding ammonia, until the greater part of the ammonia still present in the gelatine has evaporated. The 10 remaining emulsion may be neutralized by adding citric acid and may then be poured.

*Example 3*

300 grams silver nitrate are dissolved in 3000 20 ccms. distilled water. On the other hand, 210 grams potassium bromide, 7.5 grams potassium iodide and 10 grams gelatine are dissolved in another 3 litres distilled water. The silver salt solution is now entered under continuous stirring in 25 the alkali halide solution. After the silver halide has formed and settled down as a sediment, the supernatant liquid is removed by decantation and the silver bromide is washed once with distilled water and divided in two parts. The first part 30 is added under continuous stirring to a solution containing 400 grams gelatine and 100 ccms. of a 25% ammonia solution in 4500 ccms. distilled water. This mixture is kept 20 minutes at 50° C. and there is now added to it the other half of the 35 silver halide sediment together with another 100 ccms. of a 25% ammonia solution. The mixture is kept further 30 minutes at 50° C. under continuous stirring and the ammonia still present therein is neutralized with citric acid, until the 40 emulsion shows only a very slight alkaline or a neutral reaction.

According to the degree of sensitivity of the gelatine used the emulsion is allowed to age for a shorter or longer period at a suitable temperature until it has reached the optimum sensitivity, 45 when it is ready for pouring.

Obviously the individual steps, quantities, temperatures etc. described with reference to the examples may be widely varied provided only that 50 the general idea underlying the new aging method remain unchanged. This general idea consists therein, that while the emulsion is being prepared, and more especially while it is being digested, there is slowly fed to the growing silver halide grain fresh, if possible chemically pure 55 silver halide. This can be realized by gradually adding to the emulsions containing substances such as ammonia, which further the aging process, during this process further quantities of 60 washed-out silver halide having a finer grain and eventually of further substances which further the aging process, such as ammonia. In this process the finer grained silver bromide is dissolved by the ammonia present in the emulsion 65 and now recrystallizes on the larger grains of silver halide already present in the emulsion, whereby the size of these grains is gradually increased.

By proceeding in the manner described, I am 70 enabled to prepare peptisation emulsions of a relatively high order of grain size which are more sensitive to the action of light than the emulsions of a similar order of grain size produced according to customary methods, and further to 75 simplify considerably the manufacture.

Various changes may be made in the details disclosed in the foregoing specification without departing from the invention or sacrificing the advantages thereof.

I claim:—

1. The method of aging photographic peptisation emulsions which comprises mixing sedimented silver halide, which has been freed from adhering substances and emulsified in a liquid binder, with another portion of sedimented silver halide also freed from adhering substances, which has a finer grain than the aforesaid emulsified silver halide and causing the mixture to get at a suitable temperature in the presence of a substance adapted to promote the aging process. 15

2. The method of aging photographic peptisation emulsions which comprises mixing sedimented silver halide, which has been freed from adhering substances and emulsified in a liquid binder, with another portion of sedimented silver halide 20 also freed from adhering substances and emulsified in a liquid binder which portion has a finer grain than the aforesaid emulsified silver halide and causing the mixture to age at a suitable temperature in the presence of a substance adapted 25 to promote the aging process.

3. The method of aging photographic peptisation emulsions which comprises mixing sedimented silver halide, which has been freed from adhering substances and emulsified in a liquid 30 binder and aged therein, with another portion of sedimented silver halide also freed from adhering substances, which has a finer grain than the aforesaid emulsified silver halide and causing the mixture to age at a suitable temperature in 35 the presence of a substance adapted to promote the aging process.

4. The method of aging photographic peptisation emulsions which comprises mixing sedimented silver halide, which has been freed from adhering substances and emulsified in a liquid binder and aged therein, with another portion of sedimented silver halide also freed from adhering substances and emulsified in a liquid binder which portion has a finer grain than the aforesaid emulsified silver halide and causing the mixture to age at a suitable temperature in the presence of a substance adapted to promote the aging process. 45

5. The method of aging photographic peptisation emulsions which comprises mixing sedimented silver halide, which has been freed from adhering substances and emulsified in a liquid binder, with another portion of sedimented silver halide also freed from adhering substances, which 55 has a finer grain than the aforesaid emulsified silver halide and causing the mixture to age at a suitable temperature in the presence of ammonia.

6. The method of aging photographic peptisation emulsions which comprises mixing sedimented silver halide, which has been freed from adhering substances and emulsified in a liquid binder, with another portion of sedimented silver halide also freed from adhering substances, and emulsified in a liquid binder which portion has a 65 finer grain than the aforesaid emulsified silver halide and causing the mixture to age at a suitable temperature in the presence of ammonia.

7. The method of aging photographic peptisation emulsions which comprises slowly and gradually mixing sedimented silver halide, which has been freed from adhering substances and emulsified in a liquid binder, with another portion of sedimented silver halide also freed from adhering substances, which has a finer grain than the 75

aforesaid emulsified silver halide and causing the mixture to age at a suitable temperature in the presence of a substance adapted to promote the aging process.

8. The method of aging photographic peptisation emulsions which comprises slowly and gradually mixing sedimented silver halide, which has been freed from adhering substances and emulsified in a liquid binder, with another portion of

sedimented silver halide also freed from adhering substances, and emulsified in a liquid binder which portion has a finer grain than the aforesaid emulsified silver halide and causing the mixture to age at a suitable temperature in the presence of a substance adapted to promote the aging process.

5

BRUNO CLAUS.